

July 28, 1936.

A. M. McAFFEE ET AL

2,049,014

PROCESS OF IMPROVING LUBRICATING OIL

Filed March 21, 1934



A. M. McAFFEE  
L. O. CROCKETT  
INVENTORS

BY A. M. McAffee  
their ATTORNEY

## UNITED STATES PATENT OFFICE

2,049,014

## PROCESS OF IMPROVING LUBRICATING OIL

Almer M. McAfee and Lucien O. Crockett, Port Arthur, Tex., assignors, by mesne assignments, to Gulf Oil Corporation, Pittsburgh, Pa., a corporation of Pennsylvania

Application March 21, 1934, Serial No. 716,732

2 Claims. (Cl. 196—78)

This invention relates to process of improving lubricating oil; and it comprises a method in which lubricating stock is agitated for several hours with anhydrous aluminum chlorid at a temperature approaching but below that at which extensive production of lower boiling oils occurs, the temperature of treatment ranging between 300° F. and 475° F., and finishing the so treated oil by customary refining methods; all as more fully hereinafter set forth and claimed.

The most important characteristic of lubricating oil is viscosity, and the ideal lubricating oil would be one having substantially the same viscosity at all temperatures to which it is subjected in use. Such an ideal lubricating oil has never been produced from crude petroleum, and all known petroleum lubricating oils become less viscous as their temperature increases. Oils from some crudes suffer less change of viscosity with change of temperature than do oils from other crudes. It is well known, for example, that oils made from paraffinic type crudes undergo less change of viscosity with change of temperature than do oils made from naphthenic type crudes; it is also well known that the viscosity of oils made from the paraffin base crude of Pennsylvania undergo less change of viscosity with change of temperature than do oils made from paraffin base mid-continent crude. Similarly, lubricating oils made from paraffin base mid-continent crude are better in this respect than lubricating oils made from Texas coastal crude. This relation of viscosity to temperature is now usually measured and expressed in terms of viscosity index, which latter is described by Dean and Davis in "Chemical and Metallurgical Engineering" volume 36, page 618.

The object of this invention is improvement of lubricating oils, with particular respect to their viscosity indexes.

We find that by comparatively inexpensive treatment we can alter the viscosity index of various lubricating oils, that from Texas coastal crude we can produce a lubricating oil having such a viscosity index as is ordinarily found in lubricating oils produced from mid-continent crude, that from mid-continent stock we can produce an oil having a viscosity index such as that which characterizes lubricating oils

made from Pennsylvania crude, and that from Pennsylvania crude we can produce oils which are properly characterized as "Super-Pennsylvania" in every respect. In each of these cases it will be noted that by our process we produce lubricating oils characterized by viscosity indexes ordinarily characteristic of higher grade stock than that which we use.

In our process, a lubricating stock is heated for some time with a small amount of anhydrous aluminum chlorid; the mass is stirred during this treatment; and the treatment is conducted advantageously at a temperature of about 425° F. At higher temperatures, such as 600° F., a considerable proportion of the oil charged will be converted into products of lower boiling point and lower viscosity than the material operated on, and the viscosity index of the oil will be lowered instead of raised. Temperatures very materially below 425° F., say below 300° F., do not effect the desired alteration in the characteristics of the oil being treated. We find that a temperature of about 475° F. is as high as can be used for our purpose. The amount of aluminum chlorid necessary for the conduct of our process varies with the oils being treated, but ordinarily no more than 10% by weight is required with any oil. This treatment with aluminum chlorid at elevated temperature may be effected by putting all of the aluminum chlorid on the oil in one treatment, or the oil may be subjected to only a portion of the aluminum chlorid in one treatment, sludge from such treatment is then removed from the oil and partially treated oil is then subjected to further treatment with the remainder of the aluminum chlorid. This latter mode of treatment we refer to as "two-stage" treatment. In all cases the sludge is settled and separated from the oil prior to further processing. After the aluminum chlorid treatment, whether it be single stage or two-stage treatment, we charge the treated oil into a reducing still and there reduce it to the desired viscosity. We preferably use contact clay in the reducing still during the reducing operation, and we find one-half pound of clay per gallon of oil a suitable proportion.

When the term "lubricating stock" is used herein, it is used in the mode most common in the petroleum refining industry; that is, either

for a petroleum fraction characterized by such viscosity and fire test that it will produce a finished commercial lubricating oil when refined by conventional sulfuric acid treatment or by filtration through clay or other equivalent refining process for removing asphaltic components therefrom and improving the color and carbon residue test thereof, or for a petroleum fraction composed predominantly of such a material together with a minor portion of related material of adjacent boiling range which is incidentally present and which minor portion will be removed by distillation in the finishing steps. As used here the term excludes all materials other than liquid petroleum the predominant portion of which is characterized by viscosity suitable for lubricating purposes, and it specifically excludes gases and non-viscous petroleum fractions which could acquire the characteristics of lubricating oil only by conversion into totally dissimilar material as distinguished from finishing into a closely related product.

As used herein the term "lubricating stock" also excludes cracked distillates and is intended to be limited to stocks of the character set forth hereinabove, having boiling ranges above that of the fraction commonly known as gas oil.

We set out below a number of specific examples of the practice of our invention, and these specific examples include treatment of lubricating distillates from Texas coastal crude, and treatment of unfiltered bright stocks from mid-continent crudes, from a West Texas crude, and from a Pennsylvania crude.

The accompanying flow chart graphically presents our process. Referring to the flow chart, Fig. 1, reference number one represents a tank of the material with which we start. This is a lubricating stock, and is ordinarily a dewaxed or wax-free stock. The stock from tank number one is charged into treating vessel 2, which vessel is provided with an agitating device 3 driven by a motor 4, and the stock is there treated at temperatures of approximately 300° F. to 475° F., with anhydrous aluminum chlorid. Sludge from this treatment is settled out, is separately withdrawn from treating vessel 2, and is discharged from the process at 5. After sludge has been settled out, the treated oil is separately withdrawn from vessel 2 through line 6. Contact clay, ordinarily in the proportion of approximately one-half pound of clay per gallon of treated oil is introduced into the treated oil at 7. The treated oil, together with the added clay, is then passed through a heating coil 8 in furnace 9, and from there it goes to flash tower 10. The heating coil 8 and flash tower 10 comprise a reducing still, and the treated oil is there reduced to the desired viscosity. Steam is introduced into the oil during this distillation. Material distilled off during the reducing distillation is condensed in condenser 11, and it then leaves the process. The reduced treated oil leaves the reducing still through line 12, is then passed through a filter or other means 13 for removal of contained clay, and then leaves the process through line 14 as the final product of our process. The aluminum chlorid used in the treatment is fed to treating vessel 2 from a source of supply 15. In the specific examples hereinafter set forth, the lubricating stock fed to our process, if from Pennsylvania crude, has been dewaxed; if from a wax-bearing crude which also contains a substantial amount of asphaltic constituents, it has

been acid treated and dewaxed; if from a non-wax-bearing crude, the stock is charged to our process direct from the still. As a refining procedure, we prefer, if a lubricating stock requires dewaxing, that the stock be dewaxed prior to our herein disclosed process, but the prior removal of wax is dictated solely by ordinary refining considerations. Acid treatment prior to dewaxing is not essential, but merely permits more complete removal of the contained wax than would otherwise be possible at the dewaxing temperature used. We wish to emphasize that our process is an efficacious and valuable one regardless of whether the wax is removed before or after our herein disclosed treatment.

A lubricating oil distillate from Texas coastal crude (the latter being a naphthenic type crude) was treated with 98% sulphuric acid in the amount of 30 pounds of acid per barrel of oil, this being 9.2% of acid by weight. The treated oil was then washed with caustic soda and blown bright. Following are the tests on the oil before and after finishing:

Table I

|                                | Lubricating oil distillate | Treated lubricating oil | 25 |
|--------------------------------|----------------------------|-------------------------|----|
| Acid treatment (98% sulfuric): |                            |                         | 30 |
| Pounds acid used, per bbl.     |                            | 30                      |    |
| Acid used, percent by weight   |                            | 9.2                     |    |
| Treating temperature ° F.      |                            | 90                      |    |
| Yield of finished oil          |                            | 82                      |    |
| Tests:                         |                            |                         |    |
| Gravity, ° A. P. I.            | 20.6                       | 21.9                    |    |
| Viscosity, S. U. V.            |                            |                         | 35 |
| At 100° F.                     | 980                        | 843                     |    |
| At 210° F.                     | 67                         | 65                      |    |
| Viscosity index                | 15                         | 29                      |    |
| Flash, ° F.                    | 410                        | 420                     |    |
| Fire, ° F.                     | 470                        | 480                     |    |
| Pour, ° F.                     | 0                          | 0                       |    |
| Color, N. P. A.                | 2.5 dil.                   | 3                       |    |
| Carbon residue percent         | 0.18                       | 0.17                    | 40 |

The above treatment represents the usual practice in finishing this type of oil for the market. It will be observed that there has been only a slight improvement in the viscosity index and slight rise in the flash and fire tests. The carbon residue test remained practically the same.

A lubricating oil distillate from Texas coastal crude (the latter being a naphthenic type crude) was treated with 98% sulphuric acid in the amount of 42 pounds of acid per barrel of oil, this being 13% of acid by weight. The so treated oil was then charged to a reducing still together with contact clay in the amount of  $\frac{1}{2}$  pound per gallon of sour oil. The oil was then reduced with fire and bottom steam to a viscosity of 75 at 210° F.

Another lot of the same lubricating oil distillate was treated with anhydrous aluminum chlorid instead of sulfuric acid. The amount of chlorid used was 32.5 pounds per barrel of oil, this being 10% by weight. The treat was made in two stages. In the first stage, 4% by weight of aluminum chlorid was added to the distillate and this was stirred for 4 hours at a temperature of 425° F. Sludge resulting from the treatment was allowed to settle and was removed from the supernatant oil. In the second stage, the remaining portion of aluminum chlorid (6%) was added to the oil from the first stage treatment and this was then stirred for 4 hours at a temperature of 307° F. Sludge was allowed to settle and was removed from the oil. The so treated oil was charged to a reducing still together with contact clay in the 75

amount of  $\frac{1}{2}$  pound per gallon of oil. The oil was then reduced with fire and bottom steam to a viscosity of 72 at 210° F.

The following table of figures gives details of the treatments and compares the product of the sulphuric acid treatment with the product of the aluminum chlorid treatment:

Table II

|                                         | Lubricating oil distillate | Lubricating oil distillate acid treated | Lubricating oil distillate aluminum chlorid treated |
|-----------------------------------------|----------------------------|-----------------------------------------|-----------------------------------------------------|
| Acid treatment (98% sulfuric):          |                            |                                         |                                                     |
| Acid used, lbs. per bbl.                |                            | 42                                      |                                                     |
| Acid used, percent by weight            |                            | 13                                      |                                                     |
| Treating temperature, ° F.              | 121-129                    |                                         |                                                     |
| Aluminum chlorid treatment:             |                            |                                         |                                                     |
| First stage—                            |                            |                                         |                                                     |
| Chlorid used, lbs. per bbl.             |                            |                                         |                                                     |
| Chlorid used, percent by weight         |                            | 13                                      |                                                     |
| Treating temperature, ° F.              |                            | 4                                       |                                                     |
| Time of treating, hours                 |                            | 425                                     |                                                     |
| Second stage—                           |                            |                                         |                                                     |
| Chlorid used, lbs. per bbl.             |                            | 4                                       |                                                     |
| Chlorid used, percent by weight         |                            | 19.5                                    |                                                     |
| Treating temperature, ° F.              |                            | 6                                       |                                                     |
| Time of treating, hours                 |                            | 307                                     |                                                     |
| Yield of treated oil, percent           |                            | 4                                       |                                                     |
| Contact clay used, lbs. per gall        | 89.8                       | 79.1                                    |                                                     |
| Temperature of reduction, ° F.          | 0.5                        | 0.5                                     |                                                     |
| Distillate from reducing still, percent | 500                        | 500                                     |                                                     |
| Yield of reduced oil, percent           | 7.5                        | 33.5                                    |                                                     |
| Tests:                                  |                            |                                         |                                                     |
| Gravity, ° A. P. I.                     | 20.5                       | 22.1                                    |                                                     |
| Viscosity, S. U. V.—                    |                            |                                         |                                                     |
| 100° F.                                 | 1227                       | 1264                                    |                                                     |
| 210° F.                                 | 73                         | 75                                      |                                                     |
| Viscosity index                         | 13                         | 19                                      |                                                     |
| Flash, C. O. C., ° F.                   | 425                        | 435                                     |                                                     |
| Fire, C. O. C., ° F.                    | 500                        | 520                                     |                                                     |
| Pour, ° F.                              | -5                         | -5                                      |                                                     |
| Color, N. P. A.                         | 3.25 dil.                  | 2.25                                    |                                                     |
| Carbon residue, percent                 | 0.23                       | 0.14                                    |                                                     |

crude (the latter being a naphthenic type crude) was treated with aluminum chlorid in the amount of 13 pounds per barrel of oil, this being 4% by weight. The treating was done at 470° F., while stirring, and was continued 12 hours. Sludge resulting from the treatment was allowed to settle out and the treated oil was then charged to a reducing still together with contact clay in the amount of  $\frac{1}{2}$  pound per gallon of oil. The oil was then reduced with aid of fire and bottom steam to a viscosity of 75 at 210° F.

Another lot of the same oil was treated in two stages with aluminum chlorid, the first stage being for 12 hours at 470° F. while stirring with 4% of chlorid. The sludge resulting from the treatment was allowed to settle and the supernatant oil was given a second stage treatment with 6% aluminum chlorid at 307° F. for 12 hours. After again separating the sludge, the treated oil was charged to a reducing still together with contact clay in the amount of  $\frac{1}{2}$  pound per gallon of oil, and the oil was there reduced with fire and bottom steam to a viscosity of 74 at 210° F.

The foregoing two runs, giving comparable results obtained by treating lubricating oil distillate from Texas coastal crude with aluminum chlorid in a single stage at high temperature and by treating the same stock in two stages, one at high temperature and one at lower temperature, are given in Table III, below:

Table III

|                                         | Lubricating oil distillate | Lubricating oil distillate aluminum chlorid treatment | 35      |
|-----------------------------------------|----------------------------|-------------------------------------------------------|---------|
|                                         | One stage                  | Two stages                                            |         |
| Aluminum chlorid treatment:             |                            |                                                       |         |
| First stage—                            |                            |                                                       |         |
| Chlorid used, lbs. per bbl.             |                            |                                                       |         |
| Chlorid used, percent by weight         |                            | 13                                                    | 13      |
| Treating temperature, ° F.              |                            | 4                                                     | 4       |
| Time of treating, hours                 |                            | 470                                                   | 470 45  |
| Second stage—                           |                            |                                                       |         |
| Chlorid used, lbs. per bbl.             |                            |                                                       |         |
| Chlorid used, percent by weight         |                            |                                                       | 19.6    |
| Treating temperature, ° F.              |                            |                                                       | 6 50    |
| Time of treating, hours                 |                            | 307                                                   |         |
| Yield of treated oil, percent           |                            | 12                                                    |         |
| Contact clay used, lbs. per gall        |                            | 88.4                                                  | 76.0    |
| Temperature of reduction, ° F.          |                            | 0.5                                                   | 0.5     |
| Distillate from reducing still, percent |                            | 500                                                   | 500 55  |
| Yield of reduced oil, percent           |                            | 25.6                                                  | 33.0    |
| Tests:                                  |                            | 59.8                                                  | 40.3    |
| Gravity, ° A. P. I.                     | 20.3                       | 22.6                                                  | 26.0    |
| Viscosity, S. U. V.—                    |                            |                                                       |         |
| 100° F.                                 | 1462                       | 1038                                                  | 789 60  |
| 210° F.                                 | 80                         | 75                                                    | 74      |
| Viscosity index                         | 20                         | 51                                                    | 84      |
| Flash, C. O. C., ° F.                   | 430                        | 450                                                   | 400     |
| Fire, C. O. C., ° F.                    | 515                        | 535                                                   | 545     |
| Pour, ° F.                              | 0                          | -10                                                   | +5      |
| Color, N. P. A.                         | 5.25                       | 8                                                     | 2.75    |
| Carbon residue, percent                 | 0.29                       | 0.84                                                  | 0.14 65 |

In the single stage treat at high temperature, shown in the second column of Table III, it will be noted that while the viscosity index was raised from 20 to 51, the carbon residue increased from 0.29% to 0.84%. It is generally recognized that the carbon residue test of a lubricating oil should be as low as possible. We treat at high temperature with a portion of our aluminum chlorid to get an improvement in the viscosity index and 75

A lubricating oil distillate from Texas coastal

- then we treat with the remaining portion of aluminum chlorid at a lower temperature to reduce the carbon residue test and to attain further improvement in viscosity index. This two-stage treatment is not necessary with a paraffinic type oil as will be shown below. It seems to be peculiar to the naphthenic type only. It will be observed in the two-stage treatment shown in the third column of Table III that the viscosity index has been improved from 20 to 84, the latter index figure, obtained by our process in a product from Texas coastal crude, being somewhat higher than the average for lubricating oils made from paraffinic mid-continent crudes. Conforming to the general rule already mentioned, the gravity of the treated oil is considerably lighter and the flash and fire tests are considerably higher than the original oil, for approximately the same viscosity at 210° F.
- 20 A reduced mid-continent crude of paraffinic type which had been treated with sulphuric acid and dewaxed, was further treated with 98% sulphuric acid in the amount of 42 pounds per barrel of oil, this being 13.1% by weight. Sludge resulting from the treatment was settled and the sour oil was charged to a reducing still together with contact clay in the amount of  $\frac{1}{2}$  pound per gallon of oil. The oil was reduced at 500° F. with fire and bottom steam to a viscosity of 116 at 210° F.
- 25 Another lot of the same oil was treated with aluminum chlorid in the amount of 32 pounds per barrel of oil (10% by weight) at a temperature of 307° F. for twelve hours while stirring. The resulting sludge was separated from the supernatant oil, and the latter was charged to a reducing still together with  $\frac{1}{2}$  pound of contact clay per gallon of oil. The oil was reduced at 30 500° F. with fire and bottom steam to a viscosity of 88 at 210° F. The following table, relating to the two runs described in this and the next preceding paragraph, gives comparative results attained when using sulphuric acid and aluminum chlorid, separately, as treating agents.

45

Table IV

| Reduced crude—Mid-continent                 |                          |                                                  |                                                      |
|---------------------------------------------|--------------------------|--------------------------------------------------|------------------------------------------------------|
|                                             | Acid treated and dewaxed | Acid treated, dewaxed, then further acid treated | Acid treated, dewaxed, then aluminum chlorid treated |
| 50 Acid treatment (98% sulfuric):           |                          |                                                  |                                                      |
| Acid used, lbs. per bbl.                    | 42                       |                                                  |                                                      |
| Acid used, % by weight                      | 13.1                     |                                                  |                                                      |
| Treating temperature, ° F.                  | 120-124                  |                                                  |                                                      |
| 55 Aluminum chlorid treatment:              |                          |                                                  |                                                      |
| Chlorid used, pounds per bbl.               | 32                       |                                                  |                                                      |
| Chlorid used, % by weight                   | 10                       |                                                  |                                                      |
| Treating temperature, ° F.                  | 307                      |                                                  |                                                      |
| 60 Time of treating, hours.                 | 12                       |                                                  |                                                      |
| Yield of treated oil, percent.              | 86.3                     | 84.4                                             |                                                      |
| Contact clay used, lbs. per gall.           | 0.5                      | 0.5                                              |                                                      |
| Temperature of reduction, ° F.              | 500                      | 500                                              |                                                      |
| 65 Distillate from reducing still, percent. | 1.3                      | 18.3                                             |                                                      |
| Yield of reduced oil, percent.              | 82.1                     | 63.2                                             |                                                      |
| Tests:                                      |                          |                                                  |                                                      |
| Gravity, ° A. P. I.                         | 22.8                     | 24.3                                             | 28.2                                                 |
| Viscosity, S. U. V.—                        |                          |                                                  |                                                      |
| 100° F.                                     | 2356                     | 2025                                             | 941                                                  |
| 210° F.                                     | 126                      | 116                                              | 88                                                   |
| Viscosity index.                            | 76                       | 76                                               | 100                                                  |
| Flash, C. O. C., ° F.                       | 510                      | 515                                              | 495                                                  |
| Fire, C. O. C., ° F.                        | 590                      | 600                                              | 575                                                  |
| Pour, ° F.                                  | 0                        | +20                                              | +30                                                  |
| Color, N. P. A.                             | 5.0 dil.                 | 5.0                                              | 2.0                                                  |
| Carbon residue, percent.                    | 1.62                     | 1.14                                             | 0.22                                                 |

The viscosity index of the stock treated was 76, which is within the range typical of oils derived from mid-continent crudes. Further acid treating did not improve the viscosity index, but it will be observed that our aluminum chlorid treatment raised the viscosity index to 100, which is typical of oils derived from Pennsylvania crudes. At the same time, we effected an extreme reduction in the carbon residue test when using a one-stage aluminum chlorid treatment. Referring to the flash and fire tests of the aluminum chlorid treated material, it will be noted that these are somewhat lower than the original oil. But we would point out that the viscosity of the charge oil is 126 at 210° F. while the aluminum chlorid treated oil was reduced only to 88 viscosity. If the aluminum chlorid treated oil had been reduced to approximately 126 viscosity at 210° F., the flash and fire tests would have been considerably higher than those of the starting oil.

A reduced mid-continent crude, acid treated and dewaxed but of higher viscosity than that used in the runs cited in Table IV, was treated in one run with 98% sulphuric acid and in another run with aluminum chlorid. The details of treatment and the results attained are shown in Table V, below:

Table V

|                                          | Reduced crude—Mid-continent | 31                                               |                                                      |
|------------------------------------------|-----------------------------|--------------------------------------------------|------------------------------------------------------|
|                                          | Acid treated and dewaxed    | Acid treated, dewaxed, then further acid treated | Acid treated, dewaxed, then aluminum chlorid treated |
| Acid treatment (98% sulfuric):           |                             |                                                  |                                                      |
| Acid used, lbs. per bbl.                 | 42                          |                                                  |                                                      |
| Acid used, percent by weight             | 13                          |                                                  |                                                      |
| Treating temperature, ° F.               | 120-124                     |                                                  |                                                      |
| Aluminum chlorid treatment:              |                             |                                                  |                                                      |
| Chlorid used, lbs. per bbl.              |                             |                                                  | 25.7                                                 |
| Chlorid used, percent by weight          |                             |                                                  | 8                                                    |
| Treating temperature, ° F.               |                             |                                                  | 425                                                  |
| Time of treating, hours.                 |                             |                                                  | 12                                                   |
| Yield of treated oil, percent.           | 81.1                        |                                                  | 77.7                                                 |
| Contact clay used, lbs. per gall.        | 0.5                         |                                                  | 0.5                                                  |
| Temperature of reduction, ° F.           |                             |                                                  | 500                                                  |
| Distillate from reducing still, percent. |                             |                                                  | 31.6                                                 |
| Yield of reduced oil, percent.           | 77.9                        |                                                  | 43.4                                                 |
| Tests:                                   |                             |                                                  |                                                      |
| Gravity, ° A. P. I.                      | 22.1                        | 23.5                                             | 29.1                                                 |
| Viscosity, S. U. V.—                     |                             |                                                  |                                                      |
| 100° F.                                  | 3669                        | 2800                                             | 1097                                                 |
| 210° F.                                  | 162                         | 140                                              | 97                                                   |
| Viscosity index.                         | 74                          | 77                                               | 102                                                  |
| Flash, C. O. C., ° F.                    | 555                         | 545                                              | 555                                                  |
| Fire, C. O. C., ° F.                     | 640                         | 630                                              | 620                                                  |
| Pour, ° F.                               | +20                         | +25                                              | +45                                                  |
| Color, N. P. A.                          | 5.5 dil.                    | 6.25                                             | 1.75                                                 |
| Carbon residue, percent.                 | 2.1                         | 1.49                                             | 0.19                                                 |

In the runs cited in Table V our aluminum chlorid treatment has changed the viscosity-temperature relationship of an oil from mid-continent crude to that typical of an oil from Pennsylvania crude. At the same time the carbon residue test has been reduced from 2.1% to 0.19%. It will be observed that sulphuric acid changed the viscosity index and carbon residue test only slightly.

A reduced West Texas crude, from Reagan County, previously treated with sulphuric acid and dewaxed, was treated with aluminum chlorid. The details of the treatment and the results attained are tabulated in Table VI.

Table VI

|                                         | Reduced West Texas crude—Reagan County | West Texas crude—Reagan County                      |
|-----------------------------------------|----------------------------------------|-----------------------------------------------------|
|                                         | Acid treated and dewaxed               | Acid treated, dewaxed then aluminum chlorid treated |
| 10                                      |                                        |                                                     |
| Aluminum chlorid treatment:             |                                        |                                                     |
| Chlorid used, pounds per barrel         | 22                                     |                                                     |
| Chlorid used, percent by weight         | 7                                      |                                                     |
| Treating temperature, ° F               | 425                                    |                                                     |
| Time of treating, hours                 | 12                                     |                                                     |
| Yield of treated oil, percent           | 84                                     |                                                     |
| Contact clay used, pounds per gallon    | 0.5                                    |                                                     |
| Temperature of reduction, ° F           | 500                                    |                                                     |
| Distillate from reducing still, percent | 28.1                                   |                                                     |
| Yield of reduced oil, percent           | 53.0                                   |                                                     |
| Tests:                                  |                                        |                                                     |
| 20 Gravity, ° A. P. I.                  | 26.2                                   | 30.5                                                |
| Viscosity, S. U. V.—                    |                                        |                                                     |
| 100° F                                  | 1740                                   | 832                                                 |
| 210° F                                  | 118                                    | 87                                                  |
| Viscosity index                         | 92                                     | 109                                                 |
| Flash, C. O. C., ° F                    | 500                                    | 510                                                 |
| Fire, C. O. C., ° F                     | 580                                    | 585                                                 |
| Pour, ° F                               | +20                                    | +30                                                 |
| Color, N. P. A.                         | dark                                   | 2.75                                                |
| Carbon residue, percent                 | 1.71                                   | 0.12                                                |

West Texas crude from Reagan County yields lubricating oils with viscosity indexes similar to those from Pennsylvania crudes. With this particular crude, our process yields lubricating oils with viscosity indexes substantially higher than the average of lubricating oils from Pennsylvania crudes. The carbon residue test is reduced to a negligible quantity by a single stage treatment.

A reduced Pennsylvania crude oil which had been dewaxed was treated with aluminum chlorid in the amount of 27.3 pounds per barrel of oil (9% by weight) at a temperature of 400° F. for 12 hours while stirring. Sludge resulting from the treatment was settled and withdrawn, and the treated oil was charged to a reducing still together with 1/2 pound of contact clay per gallon of oil. The oil was there reduced with fire and bottom steam at 500° F. to a viscosity of 78 at 210° F. Table VII below shows the results attained:

Table VII

|                                         | Reduced Pennsylvania crude | Pennsylvania crude                     |
|-----------------------------------------|----------------------------|----------------------------------------|
|                                         | Dewaxed                    | Dewaxed, then aluminum chlorid treated |
| 50                                      |                            |                                        |
| 55                                      |                            |                                        |
| Aluminum Chlorid Treatment:             |                            |                                        |
| Chlorid used, lbs. per bbl              | 27.3                       |                                        |
| Chlorid used, percent by weight         | 9.0                        |                                        |
| Treating temperature, ° F               | 400                        |                                        |
| Time of treating, hours                 | 12                         |                                        |
| Yield of treated oil, percent           | 82.3                       |                                        |
| Contact clay used, lbs. per gall.       | 0.5                        |                                        |
| Temperature of reduction, ° F           | 500                        |                                        |
| Distillate from reducing still, percent | 18.0                       |                                        |
| Yield of reduced oil, percent           | 61.4                       |                                        |
| Tests:                                  |                            |                                        |
| 65 Gravity, ° A. P. I.                  | 25.9                       | 31.0                                   |
| Viscosity, S. U. V.—                    |                            |                                        |
| 100° F                                  | 1544                       | 590                                    |
| 210° F                                  | 116                        | 78                                     |
| Viscosity index                         | 99                         | 121                                    |
| Flash, C. O. C., ° F                    | 485                        | 425                                    |
| Fire, C. O. C., ° F                     | 560                        | 500                                    |
| Pour, ° F                               | 0                          | +10                                    |
| Color, N. P. A.                         | 6.25 dil.                  | 1.75                                   |
| Carbon residue, percent                 | 1.62                       | 0.13                                   |

It will be observed that by our process, we increased the viscosity index of this Pennsylvania oil from 99 to 121, and we lowered the carbon

residue test from 1.62% to 0.13%. Such a product could properly be characterized as Super-Pennsylvania in quality.

From the foregoing examples it is seen that the viscosity index of the oil was greatly improved in every instance. In the case of a lubricating distillate from Texas coastal crude an original viscosity index of 13 was brought up to 60 in one example, and, in another example, where a two-stage aluminum chlorid treatment was used, the 10 viscosity index was increased from 20 to 84. With the mid-continent paraffin oils the viscosity index increased from 76 to 100 in one case and, in a second case, the viscosity index increased from 74 to 102. With a stock from a West Texas crude 15 the viscosity index was raised from 92 to 109, and with a Pennsylvania stock the viscosity index was raised from 99 to 121.

With temperatures ranging from about 300° to 475°, and with varying percentages of aluminum chlorid as high as 10 per cent, the viscosity indexes of lubricating oil stocks can be greatly improved. A lubricating oil distillate from Texas coastal crude (naphthenic type crude) can be treated to a viscosity index equal to that of a lubricating oil from the very best mid-continent crudes (paraffin base), and a lubricating oil from a mid-continent crude can be treated to a viscosity index equal to a lubricating oil from a Pennsylvania crude (paraffin base). Also, a lubricating stock from a Pennsylvania crude can be treated to greatly improve its viscosity index, so that in its broader aspects my invention can be practiced with any viscous petroleum oil to improve its viscosity index.

The oil resulting from the processes described is a good lubricating oil ready for use. It is, however, not essential that the fire and steam reduction be done in the presence of contact clay. I find it advantageous to do so; but that step can be omitted and the sour oil remaining after the aluminum chlorid treatment is in that event given neutralization treatment, and is then reduced by fire and steam to the desired viscosity. The treatment with aluminum chlorid improves the color to such a degree that filtration through fuller's earth is not necessary, although it may be so filtered if desired. Should the wax content of the oil produced be considered excessive for any intended purpose it may be subjected to a conventional dewaxing operation.

The described process is applicable to any lubricating oil stock, whether in the form of reduced, crude, or a distillate therefrom.

The optimum proportion of aluminum chloride for use in our process is an amount weighing in the neighborhood of 8% to 10% as much as the oil being treated, and the optimum time of treatment from 8 hours to 12 hours. When treating at temperatures in the neighborhood of 300° F. this time can be greatly exceeded without disadvantage, but if this optimum time is greatly exceeded at higher temperatures it will result in undue loss of lubricating oil by conversion into light products. The treatment will be somewhat advantageous even for a substantially shorter period of time than the optimum, the difference being one of degree in which the desired improvement is obtained. Use of aluminum chloride in amount greatly exceeding 10% is not ordinarily either harmful or helpful except in so far as it may permit somewhat shorter time of treatment, and its use in amount much less than half of the optimum is ordinarily unproductive of the

desired effect in commercially justifiable degree.

In applying our process to naphthenic type oils we find it especially advantageous to use two-stage aluminum chlorid treatment, conducting 5 the first stage treatment at a temperature within the approximate range 400° F. to 475° F., and conducting the second stage treatment at a temperature within the approximate range 300° F. to 350° F. When treating at these temperatures, 10 all other features of our process are practiced in accordance with our more detailed disclosure above.

What we claim is:

1. A process for improving the viscosity index 15 of petroleum lubricating oil which comprises agitating a petroleum lubricating stock in the absence of any substantially lighter material with anhydrous aluminum chlorid for a number of hours at a temperature between 400° F. and 475° 20 F.; separating the so treated oil from any sludge which may result from the aluminum chlorid treatment; subjecting the separated oil to a second treatment with anhydrous aluminum chlorid at a temperature between 300° F. and 350° F.;

separating the twice treated oil from any sludge which may result from the aluminum chlorid treatment; and distilling off any low boiling product of the treatment.

2. A process for improving the viscosity index 5 of petroleum oil which comprises treating a petroleum lubricating stock in the absence of any substantially lighter material and in the absence of added HCl with anhydrous aluminum chlorid for from 4 to 12 hours at a temperature between 10 425° F. and 500° F., said treatment resulting in the conversion of a substantial part of the stock into lower boiling components and in a lowering 15 of the viscosity of the material under treatment; separating the so treated stock from any sludge which may result from the aluminum chlorid treatment; and distilling the so separated oil to remove the lower boiling components resulting 20 from the treatment and so securing a residue of lubricating oil of higher viscosity index than the untreated oil.

ALMER M. McAFFEE.  
LUCIEN O. CROCKETT.